

E. J. GREIVE,  
SURFACE DECORATING,  
APPLICATION FILED AUG. 17, 1920.

1,388,426.

Patented Aug. 23, 1921.



INVENTOR.

Edmund J. Greive

BY

*Edward E. Miller*  
ATTORNEYS

# UNITED STATES PATENT OFFICE.

EDMUND J. GREIVE, OF LOS ANGELES, CALIFORNIA.

## SURFACE-DECORATING.

1,388,426.

Specification of Letters Patent. Patented Aug. 23, 1921.

Application filed August 17, 1920. Serial No. 404,229.

To all whom it may concern:

Be it known that I, EDMUND J. GREIVE, a citizen of the United States, residing at Los Angeles, in the county of Los Angeles and 5 State of California, have invented new and useful Improvements in Surface-Decorating, of which the following is a specification.

This invention relates to surface decoration and a process of making the same, and 10 while it is of general application it is especially intended and designed for the surface decoration of caskets.

It is an object of this invention to devise a method of decorating the outer surface of a 15 casket forming a highly ornamental surface which is easily, quickly and inexpensively applied, and which, when hardened, will not crack, chip or peel from the surface to which it is applied.

20 In the drawing is shown a perspective view of a casket having an ornamental coating of the improved plastic composition.

The casket is shown at 1 as of any usual or preferred construction, preferably, of 25 wood and the coating is shown at 2.

This coating has for its base a quick drying plaster such as plaster of Paris. An adhesive material, which when dry is somewhat elastic, is mixed with the plaster in 30 order that the composition formed will stick to the surface upon which it is applied. The adhesive used is, preferably gelatin glue. In order to prevent shrinking and consequent cracking or peeling of the composition, 35 when it has set, a resinous material of thick pitch-like substance is, preferably, added to the composition. For this purpose Venice turpentine is, preferably, employed.

As a practical example of the composition 40 the following formula may be used:

Water 1 gallon.

Plaster of Paris 6 pounds.

Gelatin glue  $\frac{1}{2}$  pound.

Venice turpentine  $\frac{1}{4}$  pound.

45 In making the improved plaster composition the flakes of gelatin glue are first soaked in the water until the water has been absorbed by the flakes to form a jelly-like substance. This substance is then heated until 50 in liquid form and the plaster of Paris is then added to the liquid, the mixture being constantly stirred and maintained in a heated condition. The consistency of the mixture may be regulated by adding water if necessary, it being desired to form a composition of a consistency adapted to be read-

ily applied with a brush as a liquid coating. The turpentine is then added and the composition thoroughly mixed.

The mixture is maintained in a heated 60 condition while applying the same and is coated upon the surface to be ornamented with a brush. During application of the coating it may be brushed into an uneven surface having the ornamental ridges 3 65 formed thereon. The coating is then allowed to dry and harden, when it may be sandpapered to smooth the surface thereof.

A suitable sizing is then applied to the 70 surface of the coating in order to make it possible for a lacquer coating to stick to the surface of the composition. The lacquer coating applied to the composition is, preferably, sprayed thereon over the entire surface of the composition. This coating may 75 consist of any usual lacquer and metal powder, such as bronze or gold powder. A color coating is then applied to the entire surface of the composition, preferably, by spraying. For this purpose japan colors are used, since 80 they will not mix with the metal powder coating. If found desirable gasoline or the like may be mixed with the japan colors in order to prevent the same from drying too fast and also to allow portions of said colors 85 to be subsequently rubbed from the surface of the composition. The portions of the japan colors coating the ridges 3 are, preferably, rubbed off with a cloth saturated in turpentine or gasoline in order that the 90 metal coating upon said ridges may shine through the colored coating. If desired a finish coating of lacquer may then be applied to the entire surface of the ornamental coating in order to brighten the same. 95

It will be observed that the invention, as thus described, provides for coating wood or the like with a composition which will not peel or crack, and which may be formed into an ornamental design upon which a suitable 100 ornamental coating may be applied. When applied as a coating for caskets the invention permits of the formation of an ornamental casket without necessitating the use of usual cloth covering for the casket. 105

Various changes may be made without departing from the spirit of the invention as claimed.

What is claimed is:

1. The method of decorating surfaces 110 which consists in applying thereto an elastic coating, allowing said coating to dry, apply-

2. ing a lacquer coating containing a metallic pigment, applying a color coating, and removing the color coating from portions of the surface to allow the metal coating to shine through.

2. The method of decorating surfaces which consists in applying an elastic coating thereon, forming ridges in said coating, allowing the coating to dry, sizing the coating, 10 applying a lacquer coating containing a metallic pigment, applying a color coating, and removing the colored coating from the ridges to allow the metal coating to shine through.

15 3. The method of decorating surfaces which consists in applying an elastic coating consisting of plaster of Paris, glue,

Venice turpentine and water thereon, forming ridges in said coating, allowing said coating to dry, sand papering the coating, 20 applying a sizing thereto, applying a lacquer coating containing a metallic pigment, applying a color japan coating, and removing the colored japan coating from the ridges to allow the metal coating to shine through. 25

4. A casket having the outer surface composed of an elastic coating with ridges thereon, a metallic pigment coating covering said elastic coating, and a colored japan coating covering the metallic pigment coating except on said ridges. 30

In testimony whereof I have signed my name to this specification.

EDMUND J. GREIVE.